# EUROPEAN PATENT APPLICATION

(11) **EP 2 058 383 A1**
(43) Date of publication of application: **13.05.2009**
(21) Application number: 06843399.4
(22) Date of filing: 27.12.2006
(51) Int. Cl.: C11D 7/30, C11D 7/26, C11D 7/32, C11D 7/50, C23G 5/028

(54) **PENTAFLUOROBUTANE COMPOSITION**

(30) Priority: 28.06.2006 JP 2006178285
(71) Applicant: Kaneko Chemical Co., Ltd., Koshigaya-shi Saitama 343-0041 (JP)
(72) Inventor: KANEKO, Akiyasu, Koshigaya-shi, Saitama; 343-0041 (JP)
(74) Representative: Fiesser, Gerold Michael
(86) International application number: PCT/JP2006/326017
(87) International publication number: WO 2008/001480

(57) **Abstract**

The present invention relates to a pentafluorobutane composition which comprises 100 parts by weight of 1,1,1,3,3-pentafluorobutane and 0.01 - 10 parts by weight of at least one stabilizer selected among the following (A) to (D): (A) 3,4-epoxycyclohexenylmethyl 3',4'-epoxycyclohexenecarboxylate; (B) ε-caprolactone-modified 3,4-epoxycyclohexylmethyl 3',4'-epoxycyclohexanecarboxylate; (C) vinylcyclohexene monoxide; and (D) 1,2:8,9-diepoxylimonene.

## Description

### Technical Field

The present invention relates to a pentafluorobutane composition containing 1,1,1,3,3-pentafluorobutane, and more particularly relates to a stabilizing technique thereof.

### Background Art

Chlorine-based solvents and fluorine-based solvents have been widely used, for example, as a flux cleaner, a dry cleaning solvent, a degreasing cleaner, a buff cleaner, a resist stripper, or a solvent for removing adhesion water solvent. However, since the chlorine-based solvents have been regarded as a material responsible for groundwater contamination and the fluorine-based solvents have been regarded as a material responsible for destruction of the ozone layer, the use of the above solvents has been restricted from an environmental point of view. Accordingly, novel solvents replacing the above-described solvents have been proposed in many fields.

One of the proposed novel solvents is 1,1,1,3,3-pentafluorobutane (365 mfc, chemical formula: C₄H₅F₅). Since 1,1,1,3,3-pentafluorobutane includes no chlorine in its molecular structure and has an ozone destruction potential (ODP) of 0, a low toxicity, and a low global warming potential (GWP), this compound has superior features, that is, it is clean and is friendly to the environment. In consideration of the features described above, various types of solvents using 1,1,1,3,3-pentafluorobutane have been proposed (see Patent Documents 1 to 4).

However, 1,1,1,3,3-pentafluorobutane has a problem in that when it is used under severe conditions, such as high-temperature cleaning or steam cleaning conditions, the stability thereof is degraded due to the influence of objects to be cleaned made of metals, such as iron, zinc, aluminum, copper, and brass. Accordingly, in order to prevent the above problem, it has been proposed to add various kinds of stabilizers to 1,1,1,3,3-pentafluorobutane (see Patent Documents 5 to 9).
Patent Document 1: Japanese Patent Application Laid-open Publication No. Hei6-322394
Patent Document 2: Japanese Patent Application Laid-open Publication No. Hei7-188700
Patent Document 3: Japanese Patent Application Laid-open Publication No. 2002-241796
Patent Document 4: Japanese Patent Application Laid-open Publication No. 2003-129090
Patent Document 5: Japanese Patent Application Laid-open Publication No. Hei6-166894
Patent Document 6: Japanese Patent Application Laid-open Publication No. Hei6-166895
Patent Document 7: Japanese Patent Application Laid-open Publication No. 2000-328095
Patent Document 8: Japanese Patent Application Laid-open Publication No. Hei11-152236
Patent Document 9: Japanese Patent No. 3640661

### Disclosure of Invention

### Problems to be Solved by the Invention

However, since a sufficient stabilizing effect could not be obtained when only one of the various stabilizers thus proposed was used, at least two kinds of stabilizers have been used in combination in many cases. Accordingly, a novel stabilizer having a superior stabilizing effect to those obtained in the past has been strongly desired.

The present invention has been made in consideration of the above situation, and an object of the present invention is to stabilize a pentafluorobutane composition by a novel stabilizer which is friendly to the environment.

### Means for Solving the Problems

To this end, as a primary aspect of the present invention, there is provided a pentafluorobutane composition which comprises, with respect to 100 parts by weight of 1,1,1,3,3-pentafluorobutane:
0.01 to 10 parts by weight of at least one stabilizer selected from the following (A) to (D):
   (A) 3,4-epoxycyclohexenylmethyl-3',4'-epoxycyclohexenecarboxylate;
   (B) ε-caprolactone-modified 3,4-epoxycyclohexylmethyl 3',4'-epoxycyclohexanecarboxylate;
   (C) vinylcyclohexene monoxide; and
   (D) 1,2:8,9 diepoxylimonene.

Other advantages and features of the present invention will become clear through the specification and the accompanying drawings.

### Best Mode for Carrying Out the Invention

In accordance with this specification and the accompanying drawings, at least the following will become clear.

A pentafluorobutane composition includes, with respect to 100 parts by weight of 1,1,1,3,3-pentafluorobutane,
0.01 to 10 parts by weight of at least one stabilizer selected from the following (A) to (D):
(A) 3,4-epoxycyclohexenylmethyl-3',4'-epoxycyclohexenecarboxylate;
(B) ε-caprolactone-modified 3,4-epoxycyclohexylmethyl 3',4'-epoxycyclohexanecarboxylate;
(C) vinylcyclohexene monoxide [1,2-epoxy-4-vinylcyclohexane]; and
(D) 1,2:8,9 diepoxylimonene.

Such a pentafluorobutane composition can achieve a sufficient stability of the pentafluorobutane composition containing 1,1,1,3,3-pentafluorobutane.

A pentafluorobutane composition includes, with respect to 100 parts by weight of 1,1,1,3,3-pentafluorobutane,

0.05 to 10 parts by weight of at least one stabilizer selected from nitromethane, nitroethane, 1,3-dioxolane, trimethoxymethane, 1,1,1-trimethoxyethane, and 1,2-butyleneoxide; and
0.005 to 10 parts by weight of at least one stabilizer selected from the following (A) to (D):
(A) 3,4-epoxycyclohexenylmethyl-3',4'-epoxycyclohexenecarboxylate;
(B) ε-caprolactone-modified 3,4-epoxycyclohexylmethyl 3',4'-epoxycyclohexanecarboxylate;
(C) vinylcyclohexene monoxide; and
(D) 1,2:8,9 diepoxylimonene.

Such a pentafluorobutane composition can achieve a sufficient stability of the pentafluorobutane composition containing 1,1,1,3,3-pentafluorobutane.

A pentafluorobutane composition includes, with respect to 100 parts by weight of 1,1,1,3,3-pentafluorobutane,
0.01 to 10 parts by weight of at least one stabilizer selected from nitromethane and nitroethane; and
0.005 to 10 parts by weight of at least one stabilizer selected from the following (A) to (D):
(A) 3,4-epoxycyclohexenylmethyl-3',4'-epoxycyclohexenecarboxylate;
(B) ε-caprolactone-modified 3,4-epoxycyclohexylmethyl 3',4'-epoxycyclohexanecarboxylate;
(C) vinylcyclohexene monoxide; and
(D) 1,2:8,9 diepoxylimonene.

Such a pentafluorobutane composition can achieve a sufficient stability of the pentafluorobutane composition containing 1,1,1,3,3-pentafluorobutane.

A pentafluorobutane composition includes, with respect to 100 parts by weight of 1,1,1,3,3-pentafluorobutane,
0.01 to 10 parts by weight of at least one stabilizer selected from nitromethane and nitroethane;
0.05 to 10 parts by weight of at least one stabilizer selected from 1,3-dioxolane, trimethoxymethane, 1,1,1-trimethoxyethane, and 1,2-butyleneoxide; and
0.005 to 10 parts by weight of at least one stabilizer selected from the following (A) to (D):
(A) 3,4-epoxycyclohexenylmethyl-3',4'-epoxycyclohexenecarboxylate;
(B) ε-caprolactone-modified 3,4-epoxycyclohexylmethyl 3',4'-epoxycyclohexanecarboxylate;
(C) vinylcyclohexene monoxide; and
(D) 1,2:8,9 diepoxylimonene.

Such a pentafluorobutane composition can achieve a sufficient stability of the pentafluorobutane composition containing 1,1,1,3,3-pentafluorobutane.

In addition, in the pentafluorobutane composition described above, 30 to 97 percent by weight of 1,1,1,3,3-pentafluorobutane and 3 to 70 percent by weight of normal propyl bromide may be contained, and the total amount thereof may not be more than 100 percent by weight. When normal propyl bromide is contained in the pentafluorobutane composition as described above, a pentafluorobutane composition having a superior solvent power can be obtained.

50 to 97 percent by weight of 1,1,1,3,3-pentafluorobutane and 3 to 50 percent by weight of a propylene glycol-based solvent may be contained, and the total amount thereof may not be more than 100 percent by weight. When a propylene glycol-based solvent is contained in the pentafluorobutane composition as described above, a pentafluorobutane composition having a superior solvent power can be obtained.

In addition, in the pentafluorobutane composition described above, 50 to 90 percent by weight of 1,1,1,3,3-pentafluorobutane and 10 to 50 percent by weight of at least one of nitromethane and nitroethane may be contained, and the total amount thereof may not be more than 100 percent by weight. According to the composition described above, a pentafluorobutane composition having a superior solvent power can be obtained.

In addition, in the pentafluorobutane composition described above, 50 to 97 percent by weight of 1,1,1,3,3-pentafluorobutane and 3 to 50 percent by weight of butyl alcohol may be contained, and the total amount thereof may not be more than 100 percent by weight. When butyl alcohol is contained in the pentafluorobutane composition as described above, a pentafluorobutane composition having a superior solvent power can be obtained.

In addition, in the pentafluorobutane composition described above, 10 to 97 percent by weight of 1,1,1,3,3-pentafluorobutane and 3 to 90 percent by weight of d-limonene and/or 3-methoxybutyl acetate may be contained, and the total amount thereof may not be more than 100 percent by weight. When d-limonene and/or 3-methoxybutyl acetate is contained in the pentafluorobutane composition as described above, a pentafluorobutane composition having a superior solvent power can be obtained.

### === Outline of pentafluorobutane composition ===

A pentafluorobutane composition of the present invention is a pentafluorobutane composition which includes, with respect to 100 parts by weight of 1,1,1,3,3-pentafluorobutane: 0.01 to 10 parts by weight of at least one stabilizer selected from the following (A) to (D):
(A) 3,4-epoxycyclohexenylmethyl-3',4'-epoxycyclohexenecarboxylate;
(B) ε-caprolactone-modified 3,4-epoxycyclohexylmethyl 3',4'-epoxycyclohexanecarboxylate;
(C) vinylcyclohexene monoxide [1,2-epoxy-4-vinylcyclohexane]; and
(D) 1,2:8,9 diepoxylimonene.

The above (A) to (D) stabilizers may be contained alone or in combination in the pentafluorobutane composition. When at least one of the above stabilizers (A) to (D) is contained in the pentafluorobutane composition, a decomposition reaction caused by contact between 1,1,1,3,3-pentafluorobutane and a metal can be sufficiently suppressed, and hence the generation of gas can be suppressed. Accordingly, the pentafluorobutane composition can be used, for example, to clean various metal components.

The reason that the content of the above stabilizers (A) to (D) is set in the range of 0.01 to 10 parts by weight is as follows. That is, when the content of the above stabilizers (A) to (D) is less than 0.01 parts by weight, a sufficient stabilizing effect on 1,1,1,3,3-pentafluorobutane has not been confirmed. When the content of the above stabilizers (A) to (D) is more than 10 parts by weight, although the stabilizing effect itself is sufficient, a further effect cannot be expected and hence it is not economical.

Furthermore, in another pentafluorobutane composition of the present invention, with respect to 100 parts by weight of 1,1,1,3,3-pentafluorobutane, 0.05 to 10 parts by weight of at least one stabilizer selected from nitromethane, nitroethane, 1,3-dioxolane, trimethoxymethane, 1,1,1-trimethoxyethane, and 1,2-butyleneoxide and 0.005 to 10 parts by weight of at least one stabilizer selected from the above (A) to (D) are contained.

The above stabilizers (A) to (D) may be contained alone or in combination in the pentafluorobutane composition. In addition, as in the case described above, nitromethane, nitroethane, 1,3-dioxolane, trimethoxymethane, 1,1,1-trimethoxyethane, and 1,2-butyleneoxide may also be contained alone or in combination.

When at least one of the above stabilizers (A) to (D) is used in combination with nitromethane, nitroethane, 1,3-dioxolane, trimethoxymethane, 1,1,1-trimethoxyethane, or 1,2-butyleneoxide, a decomposition reaction caused by contact between 1,1,1,3,3-pentafluorobutane and a metal can be sufficiently suppressed, and hence the generation of gas can be suppressed. Accordingly, the pentafluorobutane composition can be used, for example, to clean various metal components. In addition, the content of the stabilizers (A) to (D) can be decreased.

The reason that the content of nitromethane, nitroethane, 1,3-dioxolane, trimethoxymethane, 1,1,1-trimethoxyethane, or 1,2-butyleneoxide is set in the range of 0.05 to 10 parts by weight is as follows. That is, when the content of nitromethane, nitroethane, 1,3-dioxolane, trimethoxymethane, 1,1,1-trimethoxyethane, or 1,2-butyleneoxide is less than 0.05 parts by weight, it is difficult to further improve the stability. On the other hand, when the content of these stabilizers is more than 10 parts by weight, although the stabilizing effect itself is sufficient, a further effect cannot be expected and hence it is not economical.

Furthermore, in another pentafluorobutane composition of the present invention, with respect to 100 parts by weight of 1,1,1,3,3-pentafluorobutane, 0.01 to 10 parts by weight of at least one stabilizer selected from nitromethane and nitroethane and 0.005 to 10 parts by weight of at least one stabilizer selected from the above (A) to (D) are contained.

The above stabilizers (A) to (D) may be contained alone or in combination in the pentafluorobutane composition. In addition, as in the case described above, nitromethane and nitroethane may also be contained alone or in combination.

When at least one of the above stabilizers (A) to (D) is used in combination with nitromethane or nitroethane, a decomposition reaction caused by contact between 1,1,1,3,3-pentafluorobutane and a metal can be sufficiently suppressed, and hence the generation of gas can be suppressed. Accordingly, the pentafluorobutane composition can be used, for example, to clean various metal components. In addition, the content of the stabilizers (A) to (D) can be decreased.

The reason that the content of nitromethane or nitroethane is set in the range of 0.01 to 10 parts by weight is as follows. That is, when the content of nitromethane or nitroethane is less than 0.01 parts by weight, it is difficult to further improve the stability. On the other hand, when the content of these stabilizers is more than 10 parts by weight, although the stabilizing effect itself is sufficient, a further effect cannot be expected and hence it is not economical.

In addition, in another pentafluorobutane composition of the present invention, with respect to 100 parts by weight of 1,1,1,3,3-pentafluorobutane, 0.01 to 10 parts by weight of at least one stabilizer selected from nitromethane and nitroethane, 0.05 to 10 parts by weight of at least one stabilizer selected from 1,3-dioxolane, trimethoxymethane, 1,1,1-trimethoxyethane, and 1,2-butyleneoxide, and 0.005 to 10 parts by weight of at least one stabilizer selected from the above stabilizers (A) to (D) are contained.

The above stabilizers (A) to (D) may be contained alone or in combination in the pentafluorobutane composition. In addition, as in the case described above, nitromethane and nitroethane may also be contained alone or in combination. In addition, also as in the case described above, 1,3-dioxolane, trimethoxymethane, 1,1,1-trimethoxyethane, and 1,2-butyleneoxide may be contained alone or in combination.

When at least one of the above stabilizers (A) to (D), nitromethane or nitroethane, and 1,3-dioxolane, trimethoxymethane, 1,1,1-trimethoxyethane, or 1,2-butyleneoxide are used in combination, a decomposition reaction caused by contact between 1,1,1,3,3-pentafluorobutane and a metal can be sufficiently suppressed, and hence the generation of gas can be suppressed. Accordingly, the pentafluorobutane composition can be used, for example, to clean various metal components. In addition, the content of the stabilizers (A) to (D) can be decreased.

The reason that the content of nitromethane or nitroethane is set in the range of 0.01 to 10 parts by weight and the reason that the content of 1,3-dioxolane, trimethoxymethane, 1,1,1-trimethoxyethane, or 1,2-butyleneoxide is set in the range of 0.05 to 10 parts by weight are as follows.

That is, when the content of nitromethane or nitroethane is less than 0.01 parts by weight, and when the content of 1,3-dioxolane, trimethoxymethane, 1,1,1-trimethoxyethane, or 1,2-butyleneoxide is less than 0.05 parts by weight, it is difficult to further improve the stability. On the other hand, when the content of these stabilizers are more than 10 parts by weight, although the stabilizing effect itself is sufficient, a further effect cannot be expected and hence it is not economical.

When two types of stabilizers, that is, nitromethane or nitroethane, and 1,3-dioxolane, trimethoxymethane, 1,1,1-trimethoxyethane, or 1,2-butyleneoxide, are mixed together, a stabilizing effect equivalent to that in the past can be obtained.

Furthermore, the pentafluorobutane composition of the present invention may have the following compositions [1] to [5] in order to improve its solvent power.
[1] A pentafluorobutane composition in which 30 to 97 percent by weight of 1,1,1,3,3-pentafluorobutane and 3 to 70 percent by weight of normal propyl bromide are contained, and in which the total amount thereof is not more than 100 percent by weight.
[2] A pentafluorobutane composition in which 50 to 97 percent by weight of 1,1,1,3,3-pentafluorobutane and 3 to 50 percent by weight of a propylene glycol-based solvent are contained, and in which the total amount thereof is not more than 100 percent by weight.
[3] A pentafluorobutane composition in which 50 to 90 percent by weight of 1,1,1,3,3-pentafluorobutane and 10 to 50 percent by weight of at least one of nitromethane and nitroethane are contained, and in which the total amount thereof is not more than 100 percent by weight.
[4] A pentafluorobutane composition in which 50 to 97 percent by weight of 1,1,1,3,3-pentafluorobutane and 3 to 50 percent by weight of butyl alcohol are contained, and in which the total amount thereof is not more than 100 percent by weight.
[5] A pentafluorobutane composition in which 10 to 97 percent by weight of 1,1,1,3,3-pentafluorobutane and 3 to 90 percent by weight of d-limonene and/or 3-methoxybutyl acetate are contained, and in which the total amount thereof is not more than 100 percent by weight.

Normal propyl bromide (also called n-propyl bromide, or 1-bromopropane, and hereinafter referred to as "NPB" in some cases) described in the above [1] is a solvent suitable to improve the solvent power of the pentafluorobutane composition containing 1,1,1,3,3-pentafluorobutane of the present invention. NPB has a relatively high KB value of 125 and is superior in degreasing cleaning. In addition, since NPB has no inflammability and is nonflammable or flame-retardant like 1,1,1,3,3-pentafluorobutane, it is not categorized in a dangerous material, so that handling thereof can be easily and safely carried out. Furthermore, since chlorine and fluorine atoms are not included in its molecular structure, the ozone depletion potential (ODP) and the global warming potential (GWP) are both low; hence, NPB has superior features, that is, it is clean and is friendly to the environment.

The reason that the content of normal propyl bromide is set in the range of 3 to 70 percent by weight is as follows. That is, when the content of normal propyl bromide is less than 3 percent by weight, the pentafluorobutane composition of the present invention cannot sufficiently improve its solvent power. On the other hand, when the content of normal propyl bromide is more than 70 percent by weight, the solvent power is excessively improved, and adverse influence may arise in some cases.

In addition, nitromethane and nitroethane, and 1,3-dioxolane, trimethoxymethane, 1,1,1-trimethoxyethane, and 1,2-butyleneoxide, which are added as stabilizers for 1,1,1,3,3-pentafluorobutane, also effectively function as stabilizers for normal propyl bromide.

In addition, like normal propyl bromide, the propylene glycol-based solvent described in the above [2] is a solvent suitable to improve the solvent power of the pentafluorobutane composition containing 1,1,1,3,3-pentafluorobutane of the present invention. The propylene glycol-based solvent used in the present invention may particularly be, for example, propylene glycol methyl ether [PM] (boiling point: 120°C, flash point: 34°C), dipropylene glycol methyl ether [DPM] (boiling point: 188°C, flash point: 79°C), tripropylene glycol methyl ether [TPM] (boiling point: 242°C, flash point: 122°C), propylene glycol n-butyl ether [PnB] (boiling point: 170°C, flash point: 62°C), dipropylene glycol n-butyl ether [DPnB] (boiling point: 229°C, flash point: 106°C), tripropylene glycol n-butyl ether (boiling point: 274°C, flash point: 138°C), propylene glycol methyl ether acetate [PMA] (boiling point: 146°C, flash point: 46.5°C), propylene glycol diacetate [PGDA] (boiling point: 190°C, flash point: 93°C), propylene glycol phenyl ether [PPh] (boiling point: 243°C, flash point: 121°C), and propylene glycol monoethyl ether acetate (boiling point: 158°C, flash point: 53°C). These propylene glycol-based solvents mentioned above may be mixed alone or in combination.

The reason that the content of the propylene glycol-based solvent is set in the range of 3 to 50 percent by weight is as follows. That is, when the content of the propylene glycol-based solvent is less than 3 percent by weight, improvement in solvent power cannot be sufficiently achieved. In addition, when the content of the propylene glycol-based solvent is more than 50 percent by weight, adverse influence, such as an inflammable problem, may arise in some cases.

In addition, nitromethane and nitroethane described in the above [3] each function as stabilizers to stabilize 1,1,1,3,3-pentafluorobutane as described above and, as normal propyl bromide and the polypropylene glycol-based solvent, each also function as solvents suitable to improve the cleaning ability of 1,1,1,3,3-pentafluorobutane. One of nitromethane and nitroethane may be contained in the pentafluorobutane composition of the present invention, or both of them may be contained in the pentafluorobutane composition of the present invention.

The reason that the content of nitromethane and/or nitroethane is set in the range of 10 to 50 percent by weight is as follows. That is, when the content of nitromethane and/or nitroethane is less than 10 percent by weight, improvement in cleaning ability is not sufficient, and a sufficient cleaning effect cannot be obtained. On the other hand, when the content of nitromethane and/or nitroethane is more than 50 percent by weight, adverse influence, such as an inflammable problem, may arise in some cases.

Butyl alcohol [CH₃(CH₂)₃OH, molecular weight: 74.12, specific gravity: 0.813 (15°C), boiling point: 117.7°C, flash point: 37°C] described in the above [4] is a solvent suitable to improve the solvent power like normal propyl bromide and propylene glycol-based solvent. The reason that the content of butyl alcohol is set in the range of 3 to 50 percent by weight is as follows. That is, when the content of butyl alcohol is less than 3 percent by weight, the pentafluorobutane composition cannot sufficiently improve its solvent power. On the other hand, when the content is more than 50 percent by weight, adverse influences, such as an inflammable problem, may arise in some cases.

D-limonene and 3-methoxybutyl acetate described in the above [5] are solvents suitable to improve the cleaning ability of 1,1,1,3,3-pentafluorobutane like normal propyl bromide, the propylene glycol-based solvent, and butyl alcohol. D-limonene and 3-methoxybutyl acetate may be contained alone or in combination.

The reason that the content of d-limonene and/or 3-methoxybutyl acetate is set in the range of 3 to 90 percent by weight is as follows. That is, when the content of d-limonene and/or 3-methoxybutyl acetate is less than 3 percent by weight, improvement in cleaning ability is not sufficient, and a sufficient cleaning effect cannot be obtained. On the other hand, when the content of d-limonene and/or 3-methoxybutyl acetate is more than 90 percent by weight, the properties of d-limonene and/or 3-methoxybutyl acetate preferentially appear, and the superior properties of 1,1,1,3,3-pentafluorobutane cannot be sufficiently utilized.

In addition, in the pentafluorobutane composition of the present invention, besides the above stabilities (A) to (D), nitromethane, nitroethane, 1,3-dioxolane, trimethoxymethane, 1,1,1-trimethoxyethane, and 1,2-butyleneoxide, another kind of stabilizer may also be contained.

### === Stabilizer ===

Next, the stabilizers (A) to (D) contained in the pentafluorobutane composition of the present invention will be described. These stabilizers (A) to (D) are epoxy compounds using peracetic acid, and are compounds having small contents of chlorine, sodium, and the like because they do not use epichlorohydrin. These stabilizers (A) to (D) will be respectively described below in detail.
(A) 3,4-Epoxycyclohexenylmethyl-3',4'-epoxycyclohexenecarboxylate [(3'-4'-Epoxycyclohexane)methyl 3'-4'-Epoxycyclohexyl-carboxylate]
   This compound (hereinafter also referred to as "stabilizer (A)") is a compound having a molecular weight of 252.3 and CAS No. [2386-87-0] and is supplied, for example, from Daicel Chemical Industries, Ltd., as "CELLOXIDE 2021P (CEL2021)" (trade name). This compound is an alicyclic epoxy resin manufactured by an epoxidation technique using peracetic acid, has a liquid form with low viscosity, and includes no halogen impurities such as chlorine. The structure of this compound is shown below.
(B) ε-Caprolactone-modified 3,4-epoxycyclohexylmethyl 3',4'-epoxycyclohexanecarboxylate [(3'-4'-Epoxycyclohexane)methyl 3'-4'-Epoxycyclohexyl-carboxylate modified ε-caprolactone]
   This compound (hereinafter also referred to as "stabilizer (B)") is supplied, for example, from Daicel Chemical Industries, Ltd., as "CELLOXIDE 2081 (CEL2081)" (trade name).
(C) Vinylcyclohexene monoxide [1,2-epoxy-4-vinylcyclohexane]
   This compound (hereinafter also referred to as "stabilizer (C)") is a compound having a molecular weight of 124.18 and CAS No. [106-86-5]. This compound is supplied, for example, from Daicel Chemical Industries, Ltd., as "CELLOXIDE 2000 (CEL2000)" (trade name).
(D) 1,2:8,9 Diepoxylimonene
   This compound (hereinafter also referred to as "stabilizer (D)") is an alicyclic diepoxy compound and is a compound having CAS No. [96-08-2]. This compound is supplied, for example, from Daicel Chemical Industries, Ltd., as "CELLOXIDE 3000 (CEL3000)" (trade name). The structure of this compound is shown below.

### === Usage ===

The main usage of the pentafluorobutane composition as described above may be, for example, a resist stripper, a flux cleaner, a degreasing cleaner for fats and oils etc., a buff cleaner, a solvent for adhesives (urethane, epoxy, silicon and the like), a dry cleaning solvent, a remover for grease, oil, wax, ink and the like, a coating solvent, an extracting agent, a cleaner for various goods made of glass, ceramic, rubber and metal and particularly for an IC component, an electric device, a precision device, an optical lens, and the like, and a draining agent.

In addition, when the pentafluorobutane composition is used as a cleaning solvent, it can be used by various cleaning methods such as hand wash, immersion, spray, ultrasonic cleaning, steam cleaning, nozzle cleaning of a loading apparatus for adhesives (urethane, epoxy, silicon and the like), and other general cleaning.

### == Stabilization Confirmation Test ===

### <Test 1>

A stabilization test of 1,1,1,3,3-pentafluorobutane by the stabilizers (A) to (D) used here will be described. In this test, a confirmation test on a stabilization effect of the stabilizers (A) to (D) according to the pentafluorobutane composition of the present invention and that of conventional stabilizers was performed. As the conventional stabilizers, nitroethane, nitromethane, 1,3-dioxolane, 1,2-butyleneoxide, trimethoxymethane, 1,1,1-trimethoxyethane, and limonene were used.

As the stabilizer (A) [3,4-epoxycyclohexenylmethyl-3',4'-epoxycyclohexenecarboxylate], "CELLOXIDE 2021P (CEL2021)" (trade name) from Daicel Chemical Industries, Ltd. was used. As the stabilizer (B) [ε-caprolactone-modified 3,4-epoxycyclohexylmethyl 3',4'-epoxycyclohexanecarboxylate], "CELLOXIDE 2081 (CEL2081)" (trade name) from Daicel Chemical Industries, Ltd. was used. As the stabilizer (C) [vinylcyclohexene monoxide [1,2-epoxy-4-vinylcyclohexanel, "CELLOXIDE 2000 (CEL2000)" (trade name) from Daicel Chemical Industries, Ltd. was used. And, as the stabilizer (D) [1,2:8,9 diepoxylimonene], "CELLOXIDE 3000 (CEL3000)" (trade name) from Daicel Chemical Industries, Ltd. was used.

Next, one part by weight of each of the stabilizers (A) to (D) and the conventional stabilizers was mixed with 100 parts by weight of 1,1,1,3,3-pentafluorobutane, so that test solutions [A1] to [A11] were prepared. 50 ml of each test solution was poured into a glass-made Erlenmeyer flask having a volume of 100 ml, and one aluminum test piece (Standard: JIS A-1100P, dimensions: 13 mm × 65 mm × 3 mm) having a surface which was well polished and which was sufficiently cleaned and dried was placed in the flask so as to be in contact with both the gas and liquid phases. Subsequently, after a reflux condenser was attached to the top of the Erlenmeyer flask, the flask was heated to the boiling temperature in a hot-water bath, and refluxed so that the test piece was brought into contact with both the gas and liquid phases. A pH-test paper was provided in the reflux condenser. After refluxing for 120 hours, the flask was allowed to cool to room temperature, and the test piece was then recovered, so that the corrosion state thereof and coloring state of the liquid phase were observed. Furthermore, a generated gas was checked by the pH-test paper.

Table 1 is the summary of the test results. As for the criterion for the state of the aluminum test piece, VG (very good) indicates [no change at all], and × indicates [gloss degradation]. As for the criterion for the state of the test solution, VG (very good) indicates [colorless and transparent solution], and × indicates [colored solution]. Furthermore, as for the gas generation, VG (very good) indicates [no generation], and × indicates [gas generation].

**-Table 1-**

| Confirmation test of stabilizing effect of stabilizers (A) to (D) | | | | | |
|---|---|---|---|---|---|
| | | Amount added (parts by weight) | State of test piece | State of test solution | Gas generation |
| A1 | nitroethane | 1 | VG | VG | × |
| A2 | nitromethane | 1 | VG | VG | × |
| A3 | 1,2-butyleneoxide | 1 | × | × | × |
| A4 | 1,3-dioxolane | 1 | × | × | × |
| A5 | trimethoxymethane | 1 | × | × | × |
| A6 | 1,1,1-trimethoxyethane | 1 | × | × | × |
| A7 | limonene | 1 | × | × | × |
| A8 | stabilizer (A) | 1 | VG | VG | VG |
| A9 | stabilizer (B) | 1 | VG | VG | VG |
| A10 | stabilizer (C) | 1 | VG | VG | VG |
| A11 | stabilizer (D) | 1 | VG | VG | VG |

As shown in Table 1, as for the test solutions [A1] and [A2] using nitroethane and nitromethane, although the states of the test piece and the test solution were superior, gas was generated. From the above results, it was confirmed that nitroethane and nitromethane are each difficult to be used alone. In addition, as for the test solutions [A3] to [A7] using 1,3-dioxolane, 1,2-butyleneoxide, trimethoxymethane, 1,1,1-trimethoxyethane, or limonene, the states of the test piece and the test solution were inferior, and gas was generated. From the above results, it was confirmed that 1,3-dioxolane, 1,2-butyleneoxide, trimethoxymethane, 1,1,1-trimethoxyethane, and limonene are each difficult to be used alone.

On the other hand, as for the test solutions [A8] to [A11] using the stabilizers (A) to (D), the state of the test piece and the test solution were both superior, and the gas generation was not confirmed. From the above results, it was confirmed that each of the stabilizers (A) to (D) can be sufficiently used alone.

### <Test 2>

A test for investigating the amount of the stabilizers (A) to (D) was performed. In this test, test solutions were prepared such that the amounts of the stabilizers (A) to (D) were set in the range of 0.001 to 10 parts by weight with respect to 100 parts by weight of 1,1,1,3,3-pentafluorobutane. Subsequently, 50 ml of each test solution was poured into a glass-made Erlenmeyer flask having a volume of 100 ml, and tests similar to those described above were performed. The states of the aluminum test piece and the test solution were observed, and the gas generation was also checked. As the stabilizers (A) to (D), "CELLOXIDE 2021P (CEL2021)" (trade name), "CELLOXIDE 2081 (CEL2081)" (trade name), "CELLOXIDE 2000 (CEL2000)" (trade name), and "CELLOXIDE 3000 (CEL3000)" (trade name) supplied from Daicel Chemical Industries, Ltd. were used.

Table 2 is the summary of the test results. As for the criterion for the state of the aluminum test piece, VG (very good) indicates [no change at all], and × indicates [gloss degradation]. As for the criterion for the state of the test solution, VG (very good) indicates [colorless and transparent solution], and × indicates [colored solution]. Furthermore, as for the gas generation, VG (very good) indicates [no generation], and × indicates [gas generation].

**-Table 2-**

| Test for investigating appropriate amount of stabilizers (A) to (D) | | | | | | | | | | | | |
|---|---|---|---|---|---|---|---|---|---|---|---|---|
| | Stabilizer (A) | | | Stabilizer (B) | | | Stabilizer (C) | | | Stabilizer (D) | | |
| Amount added (parts by weight) | State of test piece | State of test solution | Gas generation, generation | State of test piece | State of test solution | Gas generation | State of test piece | State of test solution | Gas generation | State of test piece | State of test solution | Gas generation |
| 0.001 | x | x | x | x | x | x | x | x | x | x | x | x |
| 0.005 | x | x | x | x | x | x | x | x | x | x | x | x |
| 0.01 | VG | VG | VG | VG | VG | VG | VG | VG | VG | VG | VG | VG |
| 0.05 | VG | VG | VG | VG | VG | VG | VG | VG | VG | VG | VG | VG |
| 0.08 | VG | VG | VG | VG | VG | VG | VG | VG | VG | VG | VG | VG |
| 0.1 | VG | VG | VG | VG | VG | VG | VG | VG | VG | VG | VG | VG |
| 0.3 | VG | VG | VG | VG | VG | VG | VG | VG | VG | VG | VG | VG |
| 0.5 | VG | VG | VG | VG | VG | VG | VG | VG | VG | VG | VG | VG |
| 0.8 | VG | VG | VG | VG | VG | VG | VG | VG | VG | VG | VG | VG |
| 1 | VG | VG | VG | VG | VG | VG | VG | VG | VG | VG | VG | VG |
| 3 | VG | VG | VG | VG | VG | VG | VG | VG | VG | VG | VG | VG |
| 5 | VG | VG | VG | VG | VG | VG | VG | VG | VG | VG | VG | VG |
| 8 | VG | VG | VG | VG | VG | VG | VG | VG | VG | VG | VG | VG |
| 10 | VG | VG | VG | VG | VG | VG | VG | VG | VG | VG | VG | VG |

As shown in Table 2, when the amounts of the stabilizers (A) to (D) were each set in the range of 0.001 to 0.005 parts by weight with respect to 100 parts by weight 1,1,1,3,3-pentafluorobutane, the states of the test piece and the test solution were inferior, and the gas generation was confirmed, so that it was found that a sufficient stabilizing effect on 1,1,1,3,3-pentafluorobutane could not be obtained. On the other hand, when the amounts of the stabilizers (A) to (D) were each set to 0.01 parts by weight or more with respect to 100 parts by weight of 1,1,1,3,3-pentafluorobutane, the states of the test piece and the test solution were superior, and further the gas generation was not confirmed, so that it was found that a sufficient stabilizing effect on 1,1,1,3,3-pentafluorobutane could be obtained.

### <Test 3>

A test was performed in which nitromethane, nitroethane, 1,3-dioxolane, trimethoxymethane, 1,1,1-trimethoxyethane, or 1,2-butyleneoxide was mixed. In this test, test solutions were prepared such that the stabilizers (A) to (D) in the range of 0.001 to 10 parts by weight were each added to 100 parts by weight of 1,1,1,3,3-pentafluorobutane and in addition, that the amount of each of nitromethane, nitroethane, 1,3-dioxolane, trimethoxymethane, 1,1,1-trimethoxyethane, and 1,2-butyleneoxide was set to one part by weight. Subsequently, 50 ml of each test solution thus prepared was poured into a glass-made Erlenmeyer flask having a volume of 100 ml, and tests similar to those described above were performed. The states of the aluminum test piece and the test solution were investigated, and the gas generation was also checked. As the stabilizers (A) to (D), "CELLOXIDE 2021P (CEL2021)" (trade name), "CELLOXIDE 2081 (CEL2081)" (trade name), "CELLOXIDE 2000 (CEL2000)" (trade name), and "CELLOXIDE 3000 (CEL3000)" (trade name) supplied from Daicel Chemical Industries, Ltd. were used.

Tables 3 to 8 are the summaries of the test results. As for the criterion for the state of the aluminum test piece, VG (very good) indicates [no change at all], and × indicates [gloss degradation]. As for the criterion for the state of the test solution, VG (very good) indicates [colorless and transparent solution], and × indicates [colored solution]. Furthermore, as for the gas generation, VG (very good) indicates [no generation], and × indicates [gas generation].

**-Table 3-**

| Confirmation test of stabilizing effect by mixing nitroethane | | | | | | | | | | | | | |
|---|---|---|---|---|---|---|---|---|---|---|---|---|---|
| Nitroethane amount added (parts by | Amount added (parts by test weight) | Stabilizer (A) | | | Stabilizer (B) | | | Stabilizer (C) | | | Stabilizer (D) | | |
| | | State of piece | State of test solution | Gas generation | State of piece | State of test solution | Gas generation | State of test piece | State of test solution | Gas generation | State of piece | State of test solution | Gas generation |
| 1 | 0.001 | VG | VG | x | VG | VG | x | VG | VG | x | VG | VG | x |
| 1 | 0.005 | VG | VG | VG | VG | VG | VG | VG | VG | VG | VG | VG | VG |
| 1 | 0.008 | VG | VG | VG | VG | VG | VG | VG | VG | VG | VG | VG | VG |
| 1 | 0.01 | VG | VG | VG | VG | VG | VG | VG | VG | VG | VG | VG | VG |
| 1 | 0.05 | VG | VG | VG | VG | VG | VG | VG | VG | VG | VG | VG | VG |
| 1 | 0.08 | VG | VG | VG | VG | VG | VG | VG | VG | VG | VG | VG | VG |
| 1 | 0.1 | VG | VG | VG | VG | VG | VG | VG | VG | VG | VG | VG | VG |
| 1 | 0.5 | VG | VG | VG | VG | VG | VG | VG | VG | VG | VG | VG | VG |
| 1 | 1 | VG | VG | VG | VG | VG | VG | VG | VG | VG | VG | VG | VG |
| 1 | 3 | VG | VG | VG | VG | VG | VG | VG | VG | VG | VG | VG | VG |
| 1 | 5 | VG | VG | VG | VG | VG | VG | VG | VG | VG | VG | VG | VG |
| 1 | 8 | VG | VG | VG | VG | VG | VG | VG | VG | VG | VG | VG | VG |
| 1 | 10 | VG | VG | VG | VG | VG | VG | VG | VG | VG | VG | VG | VG |

**-Table 4-**

| Confirmation test of stabilizing effect by mixing nitromethane | | | | | | | | | | | | | |
|---|---|---|---|---|---|---|---|---|---|---|---|---|---|
| Nitromethane amount added (parts by weight) | Amount added (parts by weight) piece | Stabilizer (A) | | | Stabilizer (B) | | | Stabilizer (C) | | | Stabilizer (D) | | |
| | | State of test | State of test solution | Gas generation | State of test piece | State of test solution | Gas generation | State of test piece | State of test solution | Gas generation | State of test pierce | State of test solution | Gas generation |
| 1 | 0.001 | VG | VG | x | VG | VG | x | VG | VG | x | VG | VG | x |
| 1 | 0.005 | VG | VG | VG | VG | VG | VG | VG | VG | VG | VG | VG | VG |
| 1 | 0.008 | VG | VG | VG | VG | VG | VG | VG | VG | VG | VG | VG | VG |
| 1 | 0.01 | VG | VG | VG | VG | VG | VG | VG | VG | VG | VG | VG | VG |
| 1 | 0.05 | VG | VG | VG | VG | VG | VG | VG | VG | VG | VG | VG | VG |
| 1 | 0.08 | VG | VG | VG | VG | VG | VG | VG | VG | VG | VG | VG | VG |
| 1 | 0.1 | VG | VG | VG | VG | VG | VG | VG | VG | VG | VG | VG | VG |
| 1 | 0.5 | VG | VG | VG | VG | VG | VG | VG | VG | VG | VG | VG | VG |
| 1 | 1 | VG | VG | VG | VG | VG | VG | VG | VG | VG | VG | VG | VG |
| 1 | 3 | VG | VG | VG | VG | VG | VG | VG | VG | VG | VG | VG | VG |
| 1 | 5 | VG | VG | VG | VG | VG | VG | VG | VG | VG | VG | VG | VG |
| 1 | 8 | VG | VG | VG | VG | VG | VG | VG | VG | VG | VG | VG | VG |
| 1 | 10 | VG | VG | VG | VG | VG | VG | VG | VG | VG | VG | VG | VG |

**-Table 5-**

| Confirmation test of stabilizing effect by mixing 1,3-dioxolane | | | | | | | | | | | | | |
|---|---|---|---|---|---|---|---|---|---|---|---|---|---|
| 1,3-Dioxolane amount added (parts by weight) | Amount added (parts by weight) solution | Stabilizer (A) | | | Stabilizer (B) | | | Stabilizer (C) | | | Stabilizer (D) | | |
| | | State of test piece | State of test solution | Gas test generation | State of piece | State of test solution | Gas generation | State of test piece | State of test solution | Gas generation | State of test piece | State of test solution | Gas generation |
| 1 | 0.001 | x | x | VG | x | x | VG | x | x | VG | x | x | VG |
| 1 | 0.005 | VG | VG | VG | VG | VG | VG | VG | VG | VG | VG | VG | VG |
| 1 | 0.008 | VG | VG | VG | VG | VG | VG | VG | VG | VG | VG | VG | VG |
| 1 | 0.01 | VG | VG | VG | VG | VG | VG | VG | VG | VG | VG | VG | VG |
| 1 | 0.05 | VG | VG | VG | VG | VG | VG | VG | VG | VG | VG | VG | VG |
| 1 | 0.08 | VG | VG | VG | VG | VG | VG | VG | VG | VG | VG | VG | VG |
| 1 | 0.1 | VG | VG | VG | VG | VG | VG | VG | VG | VG | VG | VG | VG |
| 1 | 0.5 | VG | VG | VG | VG | VG | VG | VG | VG | VG | VG | VG | VG |
| 1 | 1 | VG | VG | VG | VG | VG | VG | VG | VG | VG | VG | VG | VG |
| 1 | 3 | VG | VG | VG | VG | VG | VG | VG | VG | VG | VG | VG | VG |
| 1 | 5 | VG | VG | VG | VG | VG | VG | VG | VG | VG | VG | VG | VG |
| 1 | 8 | VG | VG | VG | VG | VG | VG | VG | VG | VG | VG | VG | VG |
| 1 | 10 | VG | VG | VG | VG | VG | VG | VG | VG | VG | VG | VG | VG |

**-Table 6-**

| Confirmation test of stabilizing effect by mixing trimethoxymethane | | | | | | | | | | | | | |
|---|---|---|---|---|---|---|---|---|---|---|---|---|---|
| Trimethoxy methane amount added (parts by weight) | Amount added (parts by weight) | Stabilizer (A) | | | Stabilizer (B) | | | Stabilizer (C) | | | Stabilizer (D) | | |
| | | State of test piece | State of test solution | Gas generation | State of test piece | State of testsolution | Gas generation | State of test piece | State of test solution | Gas generation | State of test piece | State of test solution | Gas generation |
| 1 | 0.001 | x | x | VG | x | x | VG | x | x | VG | x | x | VG |
| 1 | 0.005 | VG | VG | VG | VG | VG | VG | VG | VG | VG | VG | VG | VG |
| 1 | 0.008 | VG | VG | VG | VG | VG | VG | VG | VG | VG | VG | VG | VG |
| 1 | 0.01 | VG | VG | VG | VG | VG | VG | VG | VG | VG | VG | VG | VG |
| 1 | 0.05 | VG | VG | VG | VG | VG | VG | VG | VG | VG | VG | VG | VG |
| 1 | 0.08 | VG | VG | VG | VG | VG | VG | VG | VG | VG | VG | VG | VG |
| 1 | 0.1 | VG | VG | VG | VG | VG | VG | VG | VG | VG | VG | VG | VG |
| 1 | 0.5 | VG | VG | VG | VG | VG | VG | VG | VG | VG | VG | VG | VG |
| 1 | 1 | VG | VG | VG | VG | VG | VG | VG | VG | VG | VG | VG | VG |
| 1 | 3 | VG | VG | VG | VG | VG | VG | VG | VG | VG | VG | VG | VG |
| 1 | 5 | VG | VG | VG | VG | VG | VG | VG | VG | VG | VG | VG | VG |
| 1 | 8 | VG | VG | VG | VG | VG | VG | VG | VG | VG | VG | VG | VG |
| 1 | 10 | VG | VG | VG | VG | VG | VG | VG | VG | VG | VG | VG | VG |

**-Table 7-**

| Confirmation test of stabilizing effect by mixing 1,1,1-trinethoxyethane | | | | | | | | | | | | | |
|---|---|---|---|---|---|---|---|---|---|---|---|---|---|
| 1,1,1-Trimethoxyethane amount added (parts by weight) | Amount added (parts by weight) | Stabilizer (A) | | | Stabilizer (B) | | | Stabilizer (C) | | | Stabilizer (D) | | |
| | | State of test piece | State of test solution | Gas generation | State of test piece | State of test solution | Gas generation | State of test piece | State of test solution | Gasgeneration | State of test piece | State of test solution | Gas generation |
| 1 | 0.001 | x | x | VG | x | x | VG | x | x | VG | x | x | VG |
| 1 | 0.005 | VG | VG | VG | VG | VG | VG | VG | VG | VG | VG | VG | VG |
| 1 | 0.008 | VG | VG | VG | VG | VG | VG | VG | VG | VG | VG | VG | VG |
| 1 | 0.01 | VG | VG | VG | VG | VG | VG | VG | VG | VG | VG | VG | VG |
| 1 | 0.05 | VG | VG | VG | VG | VG | VG | VG | VG | VG | VG | VG | VG |
| 1 | 0.08 | VG | VG | VG | VG | VG | VG | VG | VG | VG | VG | VG | VG |
| 1 | 0.1 | VG | VG | VG | VG | VG | VG | VG | VG | VG | VG | VG | VG |
| 1 | 0.5 | VG | VG | VG | VG | VG | VG | VG | VG | VG | VG | VG | VG |
| 1 | 1 | VG | VG | VG | VG | VG | VG | VG | VG | VG | VG | VG | VG |
| 1 | 3 | VG | VG | VG | VG | VG | VG | VG | VG | VG | VG | VG | VG |
| 1 | 5 | VG | VG | VG | VG | VG | VG | VG | VG | VG | VG | VG | VG |
| 1 | 8 | VG | VG | VG | VG | VG | VG | VG | VG | VG | VG | VG | VG |
| 1 | 10 | VG | VG | VG | VG | VG | VG | VG | VG | VG | VG | VG | VG |

**-Table 8-**

| Confirmation test of stabilizing effect by mixing 1,2-butyleneoxide | | | | | | | | | | | | | |
|---|---|---|---|---|---|---|---|---|---|---|---|---|---|
| 1,2-Butyleneoxide amount added (parts by | Amount added (parts by weight) | Stabilizer (A) | | | Stabilizer (B) | | | Stabilizer (C) | | | Stabilizer (D) | | |
| | | State of test piece | State of test solution | Gas generation | State of test piece | State of test solution | Gas generation | State of test piece | State of test solution | Gasgeneration | State of test piece | State of test solution | Gas generation |
| 1 | 0.001 | x | x | VG | x | x | VG | x | x | VG | x | x | V G |
| 1 | 0.005 | VG | VG | VG | VG | VG | VG | VG | VG | VG | VG | VG | VG |
| 1 | 0.008 | VG | VG | VG | VG | VG | VG | VG | VG | VG | VG | VG | VG |
| 1 | 0.01 | VG | VG | VG | VG | VG | VG | VG | VG | VG | VG | VG | VG |
| 1 | 0.05 | VG | VG | VG | VG | VG | VG | VG | VG | VG | VG | VG | VG |
| 1 | 0.08 | VG | VG | VG | VG | VG | VG | VG | VG | VG | VG | VG | VG |
| 1 | 0.1 | VG | VG | VG | VG | VG | VG | VG | VG | VG | VG | VG | VG |
| 1 | 0.5 | VG | VG | VG | VG | VG | VG | VG | VG | VG | VG | VG | VG |
| 1 | 1 | VG | VG | VG | VG | VG | VG | VG | VG | VG | VG | VG | VG |
| 1 | 3 | VG | VG | VG | VG | VG | VG | VG | VG | VG | VG | VG | VG |
| 1 | 5 | VG | VG | VG | VG | VG | VG | VG | VG | VG | VG | VG | VG |
| 1 | 8 | VG | VG | VG | VG | VG | VG | VG | VG | VG | VG | VG | VG |
| 1 | 10 | VG | VG | VG | VG | VG | VG | VG | VG | VG | VG | VG | VG |

As shown in Tables 3 to 8, by adding nitromethane, nitroethane, 1,3-dioxolane, trimethoxymethane, 1,1,1-trimethoxyethane, or 1,2-butyleneoxide as well as each of the stabilizers (A) to (D), even when the amount of each of the stabilizers (A) to (D) was small, that is, even when the amount was in the range of 0.005 to 0.008 parts by weight, the states of the test piece and the test solution were very superior, and the gas generation was not confirmed, so that it was found that a more sufficient stabilizing effect on 1,1,1,3,3-pentafluorobutane could be obtained.

### <Test 4>

Furthermore, a test for investigating appropriate amounts of nitromethane, nitroethane, 1,3-dioxolane, trimethoxymethane, 1,1,1-trimethoxyethane, and 1,2-butyleneoxide was performed. In this test, test solutions were prepared such that the amount of each of the stabilizers (A) to (D) was set to 0.005 parts by weight with respect to 100 parts by weight of 1,1,1,3,3-pentafluorobutane and in addition, that the amount of each of nitromethane, nitroethane, 1,3-dioxolane, trimethoxymethane, 1,1,1-trimethoxyethane, and 1,2-butyleneoxide was set in the range of 0.01 to 10 parts by weight. Subsequently, 50 ml of each test solution thus prepared was poured into a glass-made Erlenmeyer flask having a volume of 100 ml, and tests similar to those described above were performed. The states of the aluminum test piece and the test solution were investigated, and the gas generation was also checked. As the stabilizers (A) to (D), "CELLOXIDE 2021P (CEL2021)" (trade name), "CELLOXIDE 2081 (CEL2081)" (trade name), "CELLOXIDE 2000 (CEL2000)" (trade name), and "CELLOXIDE 3000 (CEL3000)" (trade name) supplied from Daicel Chemical Industries, Ltd. were used.

Tables 9 to 14 are the summaries of the test results. As for the criterion for the state of the aluminum test piece, VG (very good) indicates [no change at all], and × indicates [gloss degradation]. In addition, as for the criterion for the state of the test solution, VG (very good) indicates [colorless and transparent solution], and × indicates [colored solution]. Furthermore, as for the gas generation, VG (very good) indicates [no generation], and × indicates [gas generation].

**-Table 9-**

| Test of investigating appropriate amount of nitroethane | | | | | | | | | | | | | |
|---|---|---|---|---|---|---|---|---|---|---|---|---|---|
| Nitroethane amount added (parts by weight) | Amount added (parts by weight) | Stabilizer (A) | | | Stabilizer (B) | | | Stabilizer (C) | | | Stabilizer (D) | | |
| | | State of test piece | State of test solution | Gas generation | State of test piece | State of test solution | Gas generation | State of test piece | State of test solution | Gasgeneration | State of test piece | State of test solution | Gas generation |
| 0.01 | 0.005 | VG | VG | VG | VG | VG | VG | VG | VG | VG | VG | VG | VG |
| 0.05 | 0.005 | VG | VG | VG | VG | VG | VG | VG | VG | VG | VG | VG | VG |
| 0.08 | 0.005 | VG | VG | VG | VG | VG | VG | VG | VG | VG | VG | VG | VG |
| 0.1 | 0.005 | VG | VG | VG | VG | VG | VG | VG | VG | VG | VG | VG | VG |
| 0.2 | 0.005 | VG | VG | VG | VG | VG | VG | VG | VG | VG | VG | VG | VG |
| 0.3 | 0.005 | VG | VG | VG | VG | VG | VG | VG | VG | VG | VG | VG | VG |
| 0.5 | 0.005 | VG | VG | VG | VG | VG | VG | VG | VG | VG | VG | VG | VG |
| 0.8 | 0.005 | VG | VG | VG | VG | VG | VG | VG | VG | VG | VG | VG | VG |
| 1 | 0.005 | VG | VG | VG | VG | VG | VG | VG | VG | VG | VG | VG | VG |
| 3 | 0.005 | VG | VG | VG | VG | VG | VG | VG | VG | VG | VG | VG | VG |
| 5 | 0.005 | VG | VG | VG | VG | VG | VG | VG | VG | VG | VG | VG | VG |
| 8 | 0.005 | VG | VG | VG | VG | VG | VG | VG | VG | VG | VG | VG | VG |
| 10 | 0.005 | VG | VG | VG | VG | VG | VG | VG | VG | VG | VG | VG | VG |

**-Table 10-**

| Test of investigating appropriate amount of nitromethane | | | | | | | | | | | | | |
|---|---|---|---|---|---|---|---|---|---|---|---|---|---|
| Nitromethane amount added (parts by weight) | Amount added (parts by weight) | Stabilizer(A) | | | Stabilizer (B) | | | Stabilizer (C) | | | Stabilizer (D) | | |
| | | State of test piece | State of test solution | Gas generation | State of test piece | State of test solution | Gas generation | State of test piece | State of test solution | Gasgeneration | State of test piece | State of test solution | Gas generation |
| 0.01 | 0.005 | VG | VG | VG | VG | VG | VG | VG | VG | VG | VG | VG | VG |
| 0.05 | 0.005 | VG | VG | VG | VG | VG | VG | VG | VG | VG | VG | VG | VG |
| 0.08 | 0.005 | VG | VG | VG | VG | VG | VG | VG | VG | VG | VG | VG | VG |
| 0.1 | 0.005 | VG | VG | VG | VG | VG | VG | VG | VG | VG | VG | VG | VG |
| 0.2 | 0.005 | VG | VG | VG | VG | VG | VG | VG | VG | VG | VG | VG | VG |
| 0.3 | 0.005 | VG | VG | VG | VG | VG | VG | VG | VG | VG | VG | VG | VG |
| 0.5 | 0.005 | VG | VG | VG | VG | VG | VG | VG | VG | VG | VG | VG | VG |
| 0.8 | 0.005 | VG | VG | VG | VG | VG | VG | VG | VG | VG | VG | VG | VG |
| 1 | 0.005 | VG | VG | VG | VG | VG | VG | VG | VG | VG | VG | VG | VG |
| 3 | 0.005 | VG | VG | VG | VG | VG | VG | VG | VG | VG | VG | VG | VG |
| 5 | 0.005 | VG | VG | VG | VG | VG | VG | VG | VG | VG | VG | VG | VG |
| 8 | 0.005 | VG | VG | VG | VG | VG | VG | VG | VG | VG | VG | VG | VG |
| 10 | 0.005 | VG | VG | VG | VG | VG | VG | VG | VG | VG | VG | VG | VG |

**-Table 11-**

| Test of investigating appropriate amount of 1,3-dioxolane | | | | | | | | | | | | | |
|---|---|---|---|---|---|---|---|---|---|---|---|---|---|
| 1,3-Dioxolane amount added (parts by weight) | Amount added (parts by weight) | Stabilizer (A) | | | Stabilizer (B) | | | Stabilizer (C) | | | Stabilizer (D) | | |
| | | State of test piece | State of test solution | Gas generation | State of test piece | State of test solution | Gas generation | State of test piece | State of test solution | Gasgeneration | State of test piece | State of test solution | Gas generation |
| 0.01 | 0.005 | x | x | x | x | x | x | x | x | x | x | x | x |
| 0.05 | 0.005 | VG | VG | VG | VG | VG | VG | VG | VG | VG | VG | VG | VG |
| 0.08 | 0.005 | VG | VG | VG | VG | VG | VG | VG | VG | VG | VG | VG | VG |
| 0.1 | 0.005 | VG | VG | VG | VG | VG | VG | VG | VG | VG | VG | VG | VG |
| 0.2 | 0.005 | VG | VG | VG | VG | VG | VG | VG | VG | VG | VG | VG | VG |
| 0.3 | 0.005 | VG | VG | VG | VG | VG | VG | VG | VG | VG | VG | VG | VG |
| 0.5 | 0.005 | VG | VG | VG | VG | VG | VG | VG | VG | VG | VG | VG | VG |
| 0.8 | 0.005 | VG | VG | VG | VG | VG | VG | VG | VG | VG | VG | VG | VG |
| 1 | 0.005 | VG | VG | VG | VG | VG | VG | VG | VG | VG | VG | VG | VG |
| 3 | 0.005 | VG | VG | VG | VG | VG | VG | VG | VG | VG | VG | VG | VG |
| 5 | 0.005 | VG | VG | VG | VG | VG | VG | VG | VG | VG | VG | VG | VG |
| 8 | 0.005 | VG | VG | VG | VG | VG | VG | VG | VG | VG | VG | VG | VG |
| 10 | 0.005 | VG | VG | VG | VG | VG | VG | VG | VG | VG | VG | VG | VG |

**-Table 12-**

| Test of investigating appropriate amount of trimethoxymethane | | | | | | | | | | | | | |
|---|---|---|---|---|---|---|---|---|---|---|---|---|---|
| Trimethoxy amount added (parts by weight) | Amount State piece weight) | Stabilizer (A) | | | Stabilizer (B) | | | Stabilizer (C) | | | Stabilizer (D) | | |
| | | State of test piece | State of test solution | Gas generation | State of test piece | State of test solution | Gas generation | State of test piece | State of test solution | Gasgeneration | State of test piece | State of test solution | Gas generation |
| 0.01 | 0.005 | x | x | x | x | x | x | x | x | x | x | x | x |
| 0.05 | 0.005 | VG | VG | VG | VG | VG | VG | VG | VG | VG | VG | VG | VG |
| 0.08 | 0.005 | VG | VG | VG | VG | VG | VG | VG | VG | VG | VG | VG | VG |
| 0.1 | 0.005 | VG | VG | VG | VG | VG | VG | VG | VG | VG | VG | VG | VG |
| 0.2 | 0.005 | VG | VG | VG | VG | VG | VG | VG | VG | VG | VG | VG | VG |
| 0.3 | 0.005 | VG | VG | VG | VG | VG | VG | VG | VG | VG | VG | VG | VG |
| 0.5 | 0.005 | VG | VG | VG | VG | VG | VG | VG | VG | VG | VG | VG | VG |
| 0.8 | 0.005 | VG | VG | VG | VG | VG | VG | VG | VG | VG | VG | VG | VG |
| 1 | 0.005 | VG | VG | VG | VG | VG | VG | VG | VG | VG | VG | VG | VG |
| 3 | 0.005 | VG | VG | VG | VG | VG | VG | VG | VG | VG | VG | VG | VG |
| 5 | 0.005 | VG | VG | VG | VG | VG | VG | VG | VG | VG | VG | VG | VG |
| 8 | 0.005 | VG | VG | VG | VG | VG | VG | VG | VG | VG | VG | VG | VG |
| 10 | 0.005 | VG | VG | VG | VG | VG | VG | VG | VG | VG | VG | VG | VG |

**-Table 13-**

| Test of investigating appropriate amount of 1,1,1-trimethoxyethane | | | | | | | | | | | | | |
|---|---|---|---|---|---|---|---|---|---|---|---|---|---|
| 1,1,1-Trimethoxyethane amount added (parts by weight) | Amount added (parts by weight) | Stabilizer (A) | | | Stabilizer (B) | | | Stabilizer (C) | | | Stabilizer (D) | | |
| | | State of test piece | State of test solution | Gas generation | State of test piece | State of test solution | Gas generation | State of test piece | State of test solution | Gasgeneration | State of test piece | State of test solution | Gas generation |
| 0.01 | 0.005 | x | x | x | x | x | x | x | x | x | x | x | x |
| 0.05 | 0.005 | VG | VG | VG | VG | VG | VG | VG | VG | VG | VG | VG | VG |
| 0.08 | 0.005 | VG | VG | VG | VG | VG | VG | VG | VG | VG | VG | VG | VG |
| 0.1 | 0.005 | VG | VG | VG | VG | VG | VG | VG | VG | VG | VG | VG | VG |
| 0.2 | 0.005 | VG | VG | VG | VG | VG | VG | VG | VG | VG | VG | VG | VG |
| 0.3 | 0.005 | VG | VG | VG | VG | VG | VG | VG | VG | VG | VG | VG | VG |
| 0.5 | 0.005 | VG | VG | VG | VG | VG | VG | VG | VG | VG | VG | VG | VG |
| 0.8 | 0.005 | VG | VG | VG | VG | VG | VG | VG | VG | VG | VG | VG | VG |
| 1 | 0.005 | VG | VG | VG | VG | VG | VG | VG | VG | VG | VG | VG | VG |
| 3 | 0.005 | VG | VG | VG | VG | VG | VG | VG | VG | VG | VG | VG | VG |
| 5 | 0.005 | VG | VG | VG | VG | VG | VG | VG | VG | VG | VG | VG | VG |
| 8 | 0.005 | VG | VG | VG | VG | VG | VG | VG | VG | VG | VG | VG | VG |
| 10 | 0.005 | VG | VG | VG | VG | VG | VG | VG | VG | VG | VG | VG | VG |

**-Table 14-**

| Test of investigating appropriate amount of 1,2-butyloneoxide | | | | | | | | | | | | | |
|---|---|---|---|---|---|---|---|---|---|---|---|---|---|
| 1,2- Butyleneoxide amount added (parts by test | Amount added (parts by weight) | Stabilizer (A) | | | Stabilizer (B) | | | Stabilizer (C) | | | Stabilizer (D) | | |
| | | State of test piece | State of test solution | Gas generation | State of test piece | State of test solution | Gas generation | State of test piece | State of test solution | Gasgeneration | State of test piece | State of test solution | Gas generation |
| 0.01 | 0.005 | x | x | x | x | x | x | x | x | x | x | x | x |
| 0.05 | 0.005 | VG | VG | VG | VG | VG | VG | VG | VG | VG | VG | VG | VG |
| 0.08 | 0.005 | VG | VG | VG | VG | VG | VG | VG | VG | VG | VG | VG | VG |
| 0.1 | 0.005 | VG | VG | VG | VG | VG | VG | VG | VG | VG | VG | VG | VG |
| 0.2 | 0.005 | VG | VG | VG | VG | VG | VG | VG | VG | VG | VG | VG | VG |
| 0.3 | 0.005 | VG | VG | VG | VG | VG | VG | VG | VG | VG | VG | VG | VG |
| 0.5 | 0.005 | VG | VG | VG | VG | VG | VG | VG | VG | VG | VG | VG | VG |
| 0.8 | 0.005 | VG | VG | VG | VG | VG | VG | VG | VG | VG | VG | VG | VG |
| 1 | 0.005 | VG | VG | VG | VG | VG | VG | VG | VG | VG | VG | VG | VG |
| 3 | 0.005 | VG | VG | VG | VG | VG | VG | VG | VG | VG | VG | VG | VG |
| 5 | 0.005 | VG | VG | VG | VG | VG | VG | VG | VG | VG | VG | VG | VG |
| 8 | 0.005 | VG | VG | VG | VG | VG | VG | VG | VG | VG | VG | VG | VG |
| 10 | 0.005 | VG | VG | VG | VG | VG | VG | VG | VG | VG | VG | VG | VG |

As shown in Tables 9 to 14, as for nitromethane and nitroethane, when each amount was in the range of 0.01 to 10 parts by weight, the states of the test piece and the test solution were superior, and the gas generation was not observed, so that it was confirmed that a sufficient stabilizing effect on 1,1,1,3,3-pentafluorobutane could be obtained. In addition, as for 1,3-dioxolane, trimethoxymethane, 1,1,1-trimethoxyethane, and 1,2-butyleneoxide, when each amount was in the range of 0.05 to 10 parts by weight, the states of the test piece and the test solution were superior, and the gas generation was not observed, so that it was confirmed that a sufficient stabilizing effect on 1,1,1,3,3-pentafluorobutane could be obtained.

### <Test 5>

Next, a test for investigating influence on iron and copper was performed. In this test, test solutions were prepared such that the amount of each of the stabilizers (A) to (D) was set in the range of 0.001 to 10 parts by weight with respect to 100 parts by weight of 1,1,1,3,3-pentafluorobutane. Subsequently, 50 ml of each test solution thus prepared was poured into a glass-made Erlenmeyer flask having a volume of 100 ml, and one iron test piece or one copper test piece (each having dimensions: 13 mm × 65 mm × 3 mm) each having a surface which was well polished and which was sufficiently cleaned and dried was placed in the flask so as to be in contact with both the gas and liquid phases. Next, after a reflux condenser was attached to the top of the Erlenmeyer flask, the flask was heated to the boiling temperature in a hot-water bath, and refluxed so that the test piece was brought into contact with both the gas and liquid phases. A pH-test paper was provided in the reflux condenser. After refluxing for 120 hours, the flask was allowed to cool to room temperature, and the test piece was then recovered, so that the corrosion state thereof and coloring state of the liquid phase were observed. Furthermore, a generated gas was checked by the pH-test paper. As the stabilizers (A) to (D), "CELLOXIDE 2021P (CEL2021)" (trade name), "CELLOXIDE 2081 (CEL2081)" (trade name), "CELLOXIDE 2000 (CEL2000)" (trade name), and "CELLOXIDE 3000 (CEL3000)" (trade name) supplied from Daicel Chemical Industries, Ltd. were used.

Tables 15 and 16 are the summaries of the test results. Table 15 is the summary of the cases of iron. Table 16 is the summary of the cases of copper. As for the criterion for the state of the iron or copper test piece, VG (very good) indicates [no change at all], and × indicates [gloss degradation]. As for the criterion for the state of the test solution, VG (very good) indicates [colorless and transparent solution], and × indicates [colored solution]. Furthermore, as for the gas generation, VG (very good) indicates [no generation], and × indicates [gas generation].

**-Table 15-**

| Confirmation test of influence on iron | | | | | | | | | | | | |
|---|---|---|---|---|---|---|---|---|---|---|---|---|
| | Stabilizer (A) | | | Stabilizer (B) | | | Stabilizer (C) | | | Stabilizer (D) | | |
| Amount added (parts by weight) | State of test piece | State of test solution | Gas generation | State of test piece | State of test solution | Gas generation | State of test piece | State of test solution | Gasgeneration | State of test piece | State of test solution | Gas generation |
| 0.001 | x | x | x | x | x | x | x | x | x | x | x | x |
| 0.005 | x | x | x | x | x | x | x | x | x | x | x | x |
| 0.01 | VG | VG | VG | VG | VG | VG | VG | VG | VG | VG | VG | VG |
| 0.05 | VG | VG | VG | VG | VG | VG | VG | VG | VG | VG | VG | VG |
| 0.08 | VG | VG | VG | VG | VG | VG | VG | VG | VG | VG | VG | VG |
| 0.1 | VG | VG | VG | VG | VG | VG | VG | VG | VG | VG | VG | VG |
| 0.3 | VG | VG | VG | VG | VG | VG | VG | VG | VG | VG | VG | VG |
| 0.5 | VG | VG | VG | VG | VG | VG | VG | VG | VG | VG | VG | VG |
| 0.8 | VG | VG | VG | VG | VG | VG | VG | VG | VG | VG | VG | VG |
| 1 | VG | VG | VG | VG | VG | VG | VG | VG | VG | VG | VG | VG |
| 3 | VG | VG | VG | VG | VG | VG | VG | VG | VG | VG | VG | VG |
| 5 | VG | VG | VG | VG | VG | VG | VG | VG | VG | VG | VG | VG |
| 8 | VG | VG | VG | VG | VG | VG | VG | VG | VG | VG | VG | VG |
| 10 | VG | VG | VG | VG | VG | VG | VG | VG | VG | VG | VG | VG |

**-Table 16-**

| Confirmation test of influence on copper | | | | | | | | | | | | |
|---|---|---|---|---|---|---|---|---|---|---|---|---|
| | Stabilizer (A) | | | Stabilizer (B) | | | Stabilizer (C) | | | Stabilizer (D) | | |
| Amount added (parts by weight) | State of test piece | State of test solution | Gas generation | State of test piece | State of test solution | Gas generation | State of test piece | State of test solution | Gasgeneration | State of test piece | State of test solution | Gas generation |
| 0.001 | x | x | x | x | x | x | x | x | x | x | x | x |
| 0.005 | x | x | x | x | x | x | x | x | x | x | x | x |
| 0.01 | VG | VG | VG | VG | VG | VG | VG | VG | VG | VG | VG | VG |
| 0.05 | VG | VG | VG | VG | VG | VG | VG | VG | VG | VG | VG | VG |
| 0.08 | VG | VG | VG | VG | VG | VG | VG | VG | VG | VG | VG | VG |
| 0.1 | VG | VG | VG | VG | VG | VG | VG | VG | VG | VG | VG | VG |
| 0.3 | VG | VG | VG | VG | VG | VG | VG | VG | VG | VG | VG | VG |
| 0.5 | VG | VG | VG | VG | VG | VG | VG | VG | VG | VG | VG | VG |
| 0.8 | VG | VG | VG | VG | VG | VG | VG | VG | VG | VG | VG | VG |
| 1 | VG | VG | VG | VG | VG | VG | VG | VG | VG | VG | VG | VG |
| 3 | VG | VG | VG | VG | VG | VG | VG | VG | VG | VG | VG | VG |
| 5 | VG | VG | VG | VG | VG | VG | VG | VG | VG | VG | VG | VG |
| 8 | VG | VG | VG | VG | VG | VG | VG | VG | VG | VG | VG | VG |
| 10 | VG | VG | VG | VG | VG | VG | VG | VG | VG | VG | VG | VG |

As shown in Tables 15 and 16, like the case of aluminum, when the amount of each of the stabilizers (A) to (D) was set in the range of 0.001 to 0.008 parts by weight with respect to 100 parts by weight of 1,1,1,3,3-pentafluorobutane, the states of the test piece and the test solution were inferior, and the gas generation was confirmed, so that it was found that a sufficient stabilizing effect on 1,1,1,3,3-pentafluorobutane could not be obtained. On the other hand, when the amount of each of the stabilizers (A) to (D) was 0.01 parts by weight or more with respect to 100 parts by weight of 1,1,1,3,3-pentafluorobutane, the states of the test piece and the test solution were superior, and further the gas generation was not confirmed, so that it was found that a sufficient stabilizing effect on 1,1,1,3,3-pentafluorobutane could be obtained.

### === Solvent Power Test ===

Next, a test for investigating the solvent power was performed by mixing [1] normal propyl bromide, [2] a propylene glycol-based solvent, [3] nitromethane or nitroethane, [4] butyl alcohol, or [5] d-limonene and/or 3-methoxybutyl acetate with the pentafluorobutane composition to which the stabilizer described above was added.

### <Cleaning test for machine oil>

In this test, SUS-304 test pieces (length 25 mm × width 30 mm × thickness 2 mm) were prepared, and then immersed in machine oil (CQ-30 manufactured by Nippon Oil Corporation). Each of the test pieces was immersed in each test solution for about 10 minutes. After subjecting the test piece to drying process, the state of the test piece thus cleaned was observed. As the test solutions, the solutions, which had been obtained by adding the stabilizer (A) as a stabilizer to 1,1,1,3,3-pentafluorobutane (365 mfc) and subsequently adding normal propyl bromide, propylene glycol methyl ether (PM), butyl alcohol, d-limonene, or 3-methoxybutyl acetate (3-MBA) thereto, were used. In addition, the solutions in each of which the content of nitromethane or nitroethane was increased were also prepared as the test solutions. The following Tables 17 and 18 are the summaries of the compositions of the test solutions and the cleaning results. The cleaning results are evaluated in two levels, that is, "×: low cleaning effect" and "VG (very good): superior effect".

**-Table 17-**

| Cleaning test for machine oil 1 (365mfc. NPB, PM, butyl alcohol) | | | | |
|---|---|---|---|---|
| 365mfc (percent by weight) | NPB (percent by weight) | PM (percent weight) | Butyl by alcohol (percent by weight) | Test result |
| 100 | 0 | - | - | x |
| 99 | 1 | - | - | x |
| 97 | 3 | - | - | VG |
| 95 | 5 | - | - | VG |
| 90 | 10 | - | - | VG |
| 85 | 15 | - | - | VG |
| 80 | 20 | - | - | VG |
| 75 | 25 | - | - | VG |
| 70 | 30 | - | - | VG |
| 65 | 35 | - | - | VG |
| 60 | 40 | - | - | VG |
| 50 | 50 | - | - | VG |
| 40 | 60 | - | - | VG |
| 99 | - | 1 | - | x |
| 97 | - | 3 | - | VG |
| 95 | - | 5 | - | VG |
| 90 | - | 10 | - | VG |
| 85 | - | 15 | - | VG |
| 80 | - | 20 | - | VG |
| 75 | - | 25 | - | VG |
| 70 | - | 30 | - | VG |
| 60 | - | 40 | - | VG |
| 50 | - | 50 | - | VG |
| 99 | - | - | 1 | x |
| 97 | - | - | 3 | VG |
| 95 | - | - | 5 | VG |
| 90 | - | - | 10 | VG |
| 85 | - | - | 15 | VG |
| 80 | - | - | 20 | VG |
| 75 | - | - | 25 | VG |
| 70 | - | - | 30 | VG |
| 60 | - | - | 40 | VG |
| 50 | - | - | 50 | VG |

| | | | | |
|---|---|---|---|---|
| VG: Superior effect, x: Low cleaning effect 365mfc: 1,1,1,3,3-Pentafluorobutane (C₄H₅F₅) NPB: Normal propyl bromide PM: Propylene glycol methyl ether | | | | |

**-Table 18-**

| Cleaning test for machine oil 2 (365mfc, nitroethane, nitromethane, d-limonene, 3-MBA) | | | | | |
|---|---|---|---|---|---|
| 365mfc (percent by wight) | Nitroethane (percent by weight) | Nitromethane (percent by weight) | D-limonene (percent by weight) | 3-MBA (percent by weight) | Cleaning result |
| 95 | 5 | - | - | - | x |
| 90 | 10 | - | - | - | VG |
| 80 | 20 | - | - | - | VG |
| 70 | 30 | - | - | - | VG |
| 60 | 40 | - | - | - | VG |
| 50 | 50 | - | - | - | VG |
| 95 | - | 5 | - | - | x |
| 90 | - | 10 | - | - | VG |
| 80 | - | 20 | - | - | VG |
| 70 | - | 30 | - | - | VG |
| 60 | - | 40 | - | - | VG |
| 50 | - | 50 | - | - | VG |
| 99 | - | - | 1 | | x |
| 97 | - | - | 3 | | VG |
| 95 | - | - | 5 | | VG |
| 90 | - | - | 10 | | VG |
| 80 | - | - | 20 | - | VG |
| 75 | - | - | 25 | - | VG |
| 70 | - | - | 30 | - | VG |
| 65 | - | - | 35 | - | VG |
| 60 | - | - | 40 | - | VG |
| 50 | - | - | 50 | - | VG |
| 99 | - | - | - | 1 | x |
| 97 | - | - | - | 3 | VG |
| 95 | - | - | - | 5 | VG |
| 90 | - | - | - | 10 | VG |
| 80 | - | - | - | 20 | VG |
| 75 | - | - | - | 25 | VG |
| 70 | - | - | - | 30 | VG |
| 65 | - | - | - | 35 | VG |
| 60 | - | - | - | 40 | VG |
| 50 | - | - | - | 50 | VG |

| | | | | | |
|---|---|---|---|---|---|
| VG: Superior effect, x: Low cleaning effect 365mfc: 1,1,1,3,3-Pentafluorobutane (C₄H₅F₅) 3-MBA: 3-Methoxybutyl acetate | | | | | |

From the above test results, it was confirmed that in order to obtain a sufficient cleaning ability, 10 percent by weight or more of normal propyl bromide, propylene glycol methyl ether (PM), butyl alcohol, nitromethane, or nitroethane was necessarily mixed with 1,1,1,3,3-pentafluorobutane (365 mfc). In addition, as for d-limonene and 3-methoxybutyl acetate (3-MBA), it was confirmed that 30 percent by weight or more was necessarily mixed.

### <Cleaning test for flux>

In this test, after flux (Tamura F-AL-4 manufactured by Tamura Corporation) was applied to all the surfaces of a printed-wiring boards to be used for this test and then the boards were subjected to a burning process in an electric furnace at about 200°C for about 2 minutes, each of the boards was immersed in each test solution for about 10 minutes. Then, after the printed-wiring board was subjected to a drying process, the state of the board thus cleaned was observed. As the cleaning solutions, the solutions, which had been obtained by adding the stabilizer (A) as a stabilizer to 1,1,1,3,3-pentafluorobutane (365 mfc) and subsequently adding normal propyl bromide, propylene glycol methyl ether (PM), butyl alcohol, d-limonene, or 3-methoxybutyl acetate (3-MBA), were used. In addition, the solutions in each of which the content of nitromethane or nitroethane was increased were also prepared as the test solutions. The following Tables 19 and 20 are the summaries of the compositions of the test solutions and the cleaning results. The cleaning results are evaluated in two levels, that is, "×: low cleaning effect" and "VG (very good): superior effect".

**-Table 19-**

| Cleaning test for flux 1 (365mfc, NPB, PM, butyl alcohol) | | | | |
|---|---|---|---|---|
| 365mfc (percent by weight) | NPB (percent by (percent by alcohol weight) | PM weight) | Butyl (percent by weight) | Test result |
| 100 | 0 | - | - | x |
| 90 | 10 | - | - | x |
| 80 | 20 | - | - | x |
| 70 | 30 | - | - | VG |
| 65 | 35 | - | - | VG |
| 60 | 40 | - | - | VG |
| 55 | 45 | - | - | VG |
| 50 | 50 | - | - | VG |
| 40 | 60 | - | - | VG |
| 30 | 70 | - | - | VG |
| 90 | - | 10 | - | x |
| 80 | - | 20 | - | x |
| 75 | - | 25 | - | VG |
| 70 | - | 30 | - | VG |
| 60 | - | 40 | - | VG |
| 55 | - | 45 | - | VG |
| 50 | - | 50 | - | VG |
| 40 | - | 60 | - | VG |
| 30 | - | 70 | - | VG |
| 90 | - | - | 10 | x |
| 80 | - | - | 20 | x |
| 75 | - | - | 25 | VG |
| 70 | - | - | 30 | VG |
| 60 | - | - | 40 | VG |
| 55 | - | - | 45 | VG |
| 50 | - | - | 50 | VG |
| 40 | - | - | 60 | VG |
| 30 | - | - | 70 | VG |

| | | | | |
|---|---|---|---|---|
| VG: Superior effect, x: Low cleaning effect 365mfc: 1,1,1,3,3-Pentafluorobutane (C₄H₅F₅) NPB: Normal propyl bromide PM: Propylene glycol methyl ether | | | | |

**-Table 20-**

| Cleaning test for flux 2 (365mfc, nitroethane, nitromethane, d-limonene, 3-MBA) | | | | | |
|---|---|---|---|---|---|
| 365mfc (percent by weight) | Nitroethane (percent by weight) | Nitromethane (percent by weight) | D-limonene (percent by weight) | 3-MBA (percent by weight) | Cleaning result |
| 95 | 5 | - | - | - | x |
| 90 | 10 | - | - | - | x |
| 80 | 20 | - | - | - | VG |
| 60 | 40 | - | - | - | VG |
| 50 | 50 | - | - | - | VG |
| 40 | 60 | - | - | - | VG |
| 30 | 70 | - | - | - | VG |
| 20 | 80 | - | - | - | VG |
| 95 | - | 5 | - | - | x |
| 90 | - | 10 | - | - | x |
| 80 | - | 20 | - | - | VG |
| 60 | - | 40 | - | - | VG |
| 50 | - | 50 | - | - | VG |
| 40 | - | 60 | - | - | VG |
| 30 | - | 70 | - | - | VG |
| 20 | - | 80 | - | - | VG |
| 80 | - | - | 20 | - | x |
| 70 | - | - | 30 | - | x |
| 65 | - | - | 35 | - | x |
| 60 | - | - | 40 | - | VG |
| 50 | - | - | 50 | - | VG |
| 40 | - | - | 60 | - | VG |
| 30 | - | - | 70 | - | VG |
| 20 | - | - | 80 | - | VG |
| 10 | - | - | 90 | - | VG |
| 5 | - | - | 95 | - | VG |
| 80 | - | - | - | 20 | x |
| 70 | - | - | - | 30 | x |
| 65 | - | - | - | 35 | x |
| 60 | - | - | - | 40 | VG |
| 50 | - | - | - | 50 | VG |
| 40 | - | - | - | 60 | VG |
| 30 | - | - | - | 70 | VG |
| 20 | - | - | - | 80 | VG |
| 10 | - | - | - | 90 | VG |

| | | | | | |
|---|---|---|---|---|---|
| VG: Superior effect, x: Low cleaning effect 365mfc: 1,1,1,3,3-Pentafluorobutane (C₄H₅F₅) 3-MBA: 3-Methoxybutyl acetate | | | | | |

From the above test results, it was confirmed that in order to obtain a sufficient cleaning ability, 30 percent by weight or more of normal propyl bromide was necessarily mixed with 1,1,1,3,3-pentafluorobutane (365 mfc). As for propylene glycol methyl ether (PM) and butyl alcohol, it was confirmed that 25 percent by weight or more is necessarily mixed. As for nitromethane and nitroethane, it was confirmed that 20 percent by weight or more is necessarily mixed. In addition, as for d-limonene and 3-methoxybutyl acetate (3-MBA), it was confirmed that 40 percent by weight or more was necessarily mixed.

### <Inflammability test>

In this test, since propylene glycol methyl ether (PM), butyl alcohol, nitromethane, nitroethane, d-limonene, and 3-methoxybutyl acetate (3-MBA) have inflammability and are combustible solvents, the relationship between the contents of these solvents in 1,1,1,3,3-pentafluorobutane (365 mfc) and the inflammability was investigated. The following Table 21 is the summary of the test results. In this test, the inflammability was investigated by the tag closed cup method. Since normal propyl bromide has no inflammability, it was not tested.

**-Table 21-**

| Inflammability test (365mfc, PM, butyl alcohol, nitroethane, nitromethane, d-limonene, 3-MBA) | | | | | | | |
|---|---|---|---|---|---|---|---|
| 365mfc (percent by weight) | PM (percent by weight) | Butyl alcohol (percent by weight) | Nitroethane (percent by weight) | Nitromethane (percent by weight) | D-limonene (percent by weight) | 3-MBA (percent by weight) | Inflammability |
| 70 | 30 | - | - | - | - | - | No |
| 60 | 40 | - | - | - | - | - | No |
| 50 | 50 | - | - | - | - | - | No |
| 40 | 60 | - | - | - | - | - | Yes |
| 30 | 70 | - | - | - | - | - | Yes |
| 20 | 80 | - | - | - | - | - | Yes |
| 10 | 90 | - | - | - | - | - | Yes |
| 70 | - | 30 | - | - | - | - | No |
| 60 | - | 40 | - | - | - | - | No |
| 50 | - | 50 | - | - | - | - | No |
| 40 | - | 60 | - | - | - | - | Yes |
| 30 | - | 70 | - | - | - | - | Yes |
| 20 | - | 80 | - | - | - | - | Yes |
| 10 | - | 90 | - | - | - | - | Yes |
| 70 | - | - | 30 | - | - | - | No |
| 60 | - | - | 40 | - | - | - | No |
| 50 | - | - | 50 | - | - | - | No |
| 40 | - | - | 60 | - | - | - | Yes |
| 30 | - | - | 70 | - | - | - | Yes |
| 20 | - | - | 80 | - | - | - | Yes |
| 10 | - | - | 90 | - | - | - | Yes |
| 70 | - | - | - | 30 | - | - | No |
| 60 | - | - | - | 40 | - | - | No |
| 50 | - | - | - | 50 | - | - | No |
| 40 | - | - | - | 60 | - | - | Yes |
| 30 | - | - | - | 70 | - | - | Yes |
| 20 | - | - | - | 80 | - | - | Yes |
| 10 | - | - | - | 90 | - | - | Yes |
| 70 | - | - | - | - | 30 | - | No |
| 60 | - | - | - | - | 40 | - | No |
| 50 | - | - | - | - | 50 | - | No |
| 40 | - | - | - | - | 60 | - | No |
| 30 | - | - | - | - | 70 | - | No |
| 20 | - | - | - | - | 80 | - | No |
| 10 | - | - | - | - | 90 | - | No |
| 5 | - | - | - | - | 95 | - | Yes |
| 70 | - | - | - | - | - | 30 | No |
| 60 | - | - | - | - | - | 40 | No |
| 50 | - | - | - | - | - | 50 | No |
| 40 | - | - | - | - | - | 60 | No |
| 30 | - | - | - | - | - | 70 | No |
| 20 | - | - | - | - | - | 80 | No |
| 10 | - | - | - | - | - | 90 | No |
| 5 | - | - | - | - | - | 95 | Yes |

| | | | | | | | |
|---|---|---|---|---|---|---|---|
| 365mfc: 1,1,1,3,3-Pentafluorobutane PM: Propylene glycol methyl ether 3-MBA: 3-methoxybutyl acetate | | | | | | | |

From the above test results, in order to make the test solutions noninflammable, it was confirmed that the content of propylene glycol methyl ether (PM), butyl alcohol, nitromethane, or nitroethane should be 50 percent by weight or less with respect to 1,1,1,3,3-pentafluorobutane (365 mfc). In addition, it was confirmed that the content of d-limonene or 3-methoxybutyl acetate (3-MBA) should be 90 percent by weight or less.

## Claims

1. A pentafluorobutane composition comprising, with respect to 100 parts by weight of 1,1,1,3,3-pentafluorobutane,
0.01 to 10 parts by weight of at least one stabilizer selected from the following (A) to (D):
(A) 3,4-epoxycyclohexenylmethyl-3',4'-epoxycyclohexenecarboxylate;
(B) ε-caprolactone-modified 3,4-epoxycyclohexylmethyl 3',4'-epoxycyclohexanecarboxylate;
(C) vinylcyclohexene monoxide; and
(D) 1,2:8,9 diepoxylimonene.

2. A pentafluorobutane composition comprising, with respect to 100 parts by weight of 1,1,1,3,3-pentafluorobutane,
0.05 to 10 parts by weight of at least one stabilizer selected from nitromethane, nitroethane, 1,3-dioxolane, trimethoxymethane, 1,1,1-trimethoxyethane, and 1,2-butyleneoxide; and
0.005 to 10 parts by weight of at least one stabilizer selected from the following (A) to (D):
(A) 3,4-epoxycyclohexenylmethyl-3',4'-epoxycyclohexenecarboxylate;
(B) ε-caprolactone-modified 3,4-epoxycyclohexylmethyl 3',4'-epoxycyclohexanecarboxylate;
(C) vinylcyclohexene monoxide; and
(D) 1,2:8,9 diepoxylimonene.

3. A pentafluorobutane composition comprising, with respect to 100 parts by weight of 1,1,1,3,3-pentafluorobutane,
0.01 to 10 parts by weight of at least one stabilizer selected from nitromethane and nitroethane; and
0.005 to 10 parts by weight of at least one stabilizer selected from the following (A) to (D):
(A) 3,4-epoxycyclohexenylmethyl-3',4'-epoxycyclohexenecarboxylate;
(B) ε-caprolactone-modified 3,4-epoxycyclohexylmethyl 3',4'-epoxycyclohexanecarboxylate;
(C) vinylcyclohexene monoxide; and
(D) 1,2:8,9 diepoxylimonene.

4. A pentafluorobutane composition comprising, with respect to 100 parts by weight of 1,1,1,3,3-pentafluorobutane,
0.01 to 10 parts by weight of at least one stabilizer selected from nitromethane and nitroethane;
0.05 to 10 parts by weight of at least one stabilizer selected from 1,3-dioxolane, trimethoxymethane, 1,1,1-trimethoxyethane, and 1,2-butyleneoxide; and
0.005 to 10 parts by weight of at least one stabilizer selected from the following (A) to (D):
(A) 3,4-epoxycyclohexenylmethyl-3',4'-epoxycyclohexenecarboxylate;
(B) ε-caprolactone-modified 3,4-epoxycyclohexylmethyl 3',4'-epoxycyclohexanecarboxylate;
(C) vinylcyclohexene monoxide; and
(D) 1,2:8,9 diepoxylimonene.

5. The pentafluorobutane composition according to any one of claims 1 to 4, wherein 30 to 97 percent by weight of 1,1,1,3,3-pentafluorobutane and 3 to 70 percent by weight of normal propyl bromide are contained, and the total amount thereof is not more than 100 percent by weight.

6. The pentafluorobutane composition according to any one of claims 1 to 4, wherein 50 to 97 percent by weight of 1,1,1,3,3-pentafluorobutane and 3 to 50 percent by weight of a propylene glycol-based solvent are contained, and the total amount thereof is not more than 100 percent by weight.

7. The pentafluorobutane composition according to claim 1, wherein 50 to 90 percent by weight of 1,1,1,3,3-pentafluorobutane and 10 to 50 percent by weight of at least one of nitromethane and nitroethane are contained, and the total amount thereof is not more than 100 percent by weight.

8. The pentafluorobutane composition according to any one of claims 1 to 4, wherein 50 to 97 percent by weight of 1,1,1,3,3-pentafluorobutane and 3 to 50 percent by weight of butyl alcohol are contained, and the total amount thereof is not more than 100 percent by weight.

9. The pentafluorobutane composition according to any one of claims 1 to 4, wherein 10 to 97 percent by weight of 1,1,1,3,3-pentafluorobutane and 3 to 90 percent by weight of d-limonene and/or 3-methoxybutyl acetate are contained, and the total amount thereof is not more than 100 percent by weight.
